

## UNITED STATES PATENT OFFICE

JAMES MORTON, OF EDINBURGH, SCOTLAND, AND JAMES IVOR MORGAN JONES, OF LANCASTER, ENGLAND, ASSIGNORS TO MORTON SUNDOUR FABRICS, LIMITED, OF CARLISLE, ENGLAND

## DYEING AND PRINTING

No Drawing. Application filed April 18, 1929, Serial No. 356,300, and in Great Britain April 26, 1928.

This invention relates to dyeing and printing, and more particularly to processes in which vat colours are employed.

The production of patterns with vat colours in connection with vat grounds or vat cover-prints or the like is usually or may be effected by two methods:—

(1) First dyeing or printing the ground, and then overprinting with a suitable mixture containing an illuminating colour which effects a discharging of the ground or first print, while fixing the illuminating colour.

(2) First printing the illuminating colour in suitable mixture, then padding or overprinting with a suitable mixture such that on developing, a preferential development of the illuminating colour occurs at the points where both colours coincide.

Both these processes present considerable difficulty, and are limited in application in so far as the number of vat dyestuffs suitable for use as illuminating colours, or otherwise, is limited.

The object of the present invention is to provide an improved or modified process particularly directed to the production of fast prints in resist styles, especially the production of resists under vat colours.

The invention consists in a process comprising the use of printing or dyeing mixtures containing enolic ethereal salts of vat dyes together with excess of oxidizing agent capable of acting as a resist towards vat colours, and having substantially no effect on the enolic ethereal salt during the processes used for fixing the vat colours, and a suitable thickening, with or without the addition of substances which assist the resisting of the vat colour in a mechanical manner.

The invention also consists in a process according to the preceding paragraph, in which the printing or dyeing mixture contains agents which whilst substantially inert as regards the enolic ethereal salt during the printing or fixing of the vat colour are yet capable of causing the development of the enolic ethereal salt by further treatment (for example, with acids; such a substance is sodium nitrite), the dyeing or printing mixture containing the enolic ethereal salt being

applied for instance to the woven fabric itself, or to the yarn prior to weaving, in which latter case it may often be conveniently incorporated with the sizing mixtures and applied to the warp or the weft or to the warp and weft as desired.

The invention also consists in processes such as those indicated below, and in products when made by those processes or by the obvious chemical equivalents thereof.

There are four principal methods by which the invention may be applied. These are as follows, references to parts being to parts by weight:—

## Case 1 65

Cloth is printed with a colour mixture containing the selected oxidizing agent together with an enolic ethereal salt of a vat dyestuff, a suitable thickening, then steamed and overprinted with an ordinary vat dye, and re-steamed to fix the vat dye. Thereafter, the cloth is subjected to the usual processes for fixation and development. Examples 1 and 2 below illustrate this case:— 75

## EXAMPLE 1

According to this example a printing mixture is made as follows:—

|                                                                                              | Parts |
|----------------------------------------------------------------------------------------------|-------|
| Soledon jade green paste (enolic ethereal salt of caledon jade green, colour index No. 1101) | 80    |
| Sodium nitrite                                                                               | 20    |
| Sodium meta nitrobenzene sulphonate                                                          | 2     |
| Soluble oil                                                                                  | 30    |
| British gum thickening                                                                       | 2     |
|                                                                                              | 46    |

This mixture is printed, dried and steamed, and then overprinted or padded with a suitable or ordinary vat printing colour, for example:— 90

|                                                                             | Parts |
|-----------------------------------------------------------------------------|-------|
| Caledon red, B. N. (anthraquinone-1:2-naphthacridone—Colour Index No. 1162) | 30    |
| Glycerine                                                                   | 8     |
| British gum thickening 1:1                                                  | 35    |
| Potassium carbonate                                                         | 12    |
| Sodium formaldehyde sulphoxylate 1:1                                        | 15    |
|                                                                             | 100   |

After overprinting, the material is dried 100

and steamed with air-free steam. After steaming, the colours are developed by passing the cloth in open width or other form, through a bath containing for example:—

5 Commercial sulphuric acid 148° Tw. 10  
Parts  
Sodium bichromate 2

per 1000 parts at 30° C. followed by rinsing, soaping at the boil, and rinsing again.

10 The result is that where the red vat printing colour falls on the green resist colour, the development of the red is substantially inhibited without substantially affecting the green.

#### EXAMPLE 2

15 According to this example, a printing colour is made of the following composition:—

Parts  
15 Indigosol red H. R. (sodium salt of the disulphuric ether of leuco-helindone red R) 9  
20 Ammonium sulphocyanide 3  
Sodium chlorate 1.5  
Ammonium vanadate 1:1000 10  
25 Sodium meta nitrobenzene sulphonate 15  
Water and British gum thickening 61.5

The colour is printed, dried and steamed, then overprinted with the vat colour made as described in Example 1, in which the Caledon red B. N. is replaced by Caledon jade green. The print is then dried, steamed and developed in a bath containing for example:—

Parts  
30 Sodium bichromate 2  
35 Acetic acid 60% 5

per 1000 parts, followed by rinsing and soaping. Development of the green is substantially inhibited where it falls on the red.

#### Case 2

40 Cloth is printed and steamed as in Case 1, but instead of being overprinted, is padded with a vat dye solution in known manner.

45 Illustrations of this method are given below in Examples 3 and 4.

#### EXAMPLE 3

A printing mixture is made as follows:—

Parts  
45 Soledon jade green 20  
Sodium meta nitrobenzene sulphonate 50  
Soluble oil 2  
British gum thickening 48

50 The mixture is printed, dried and steamed, then padded in known manner with the following solution:—

Parts  
55 Caledon red B. N. (Colour Index No. 1162) 20  
60 Water 500  
Caustic soda 76° Tw. 5  
Sodium hydrosulphite 2  
Glue solution 5% 60

65 Water to 1000

After padding, the material is passed through a 1% solution of sodium bichromate in 1% sulphuric acid at 60° C., then rinsed and soaped at the boil.

79

#### EXAMPLE 4

According to this example, the cloth is printed with the following mixture and steamed:—

Parts  
15 Indigosol orange H. R. (sodium salt of the s-disulphuric ether of leuco-helindone orange R) 100  
20 Water 215  
Starch gum tragacanth thickening 450  
Ammonium sulphocyanide 30  
Sodium chlorate 25  
Ammonium vanadate 1:100 100  
25 Glycerine 30  
Sodium benzylsulphanilate 1:1 50  
Sodium m-nitrobenzene sulphonate 250  
1250  
90

After steaming, the cloth may be padded with the following mixture:—

Parts  
15 Caledon brilliant purple R. R. (Colour Index No. 1104) 50  
20 Gum Arabic 1:1 150  
Water 150  
Glycerine 100  
Potassium carbonate 150  
Water 320  
25 Rongalite C (sodium formaldehyde sulphonate. [NaHSO<sub>2</sub>.CH<sub>2</sub>O.]) 80  
1000  
105

After padding, the cloth is dried, steamed for five minutes, at 100° C., in air-free steam, and colours developed by passing through a 1% solution of sodium bichromate in 1% sulphuric acid at 60° C., followed by rinsing and soaping.

#### Case 3

The third method of applying the invention consists in applying the mixture of a selected oxidizing agent and an enolic ethereal salt of a vat dyestuff, incorporated with a suitable size or adhesive if necessary, to yarn in the form of warps or hank, such yarn being subsequently woven with untreated yarn, and the resulting cloth overprinted with an ordinary vat dyestuff as described above under Case 1 of applying the invention.

115 The following examples illustrate this case:—

#### EXAMPLE 5

120 Yarn in the form of beamed warps is treat-

125

130

ed on a sizing machine of the usual slasher type, with a mixture made as follows:—

326 parts— Size  
5 180 parts— Sodium m-nitrobenzene sulphonate  
67 parts— Soledon jade green

*Sizing mixture*

10 2800 parts— Water  
550 parts— Farina  
330 parts— I. C. starch  
275 parts— Tallow  
7.7 parts— Gum Arabic  
15 1.9 parts— Soap

The warps are then steamed either before or after weaving into cloth. If it is desired to steam before weaving, the warps as they leave the sizing machine may be wound on a 20 perforated beam such as is commonly used in beam dyeing machines.

The cloth may be woven with a figured pattern with the usual jacquard or other selecting mechanism, and may then be printed with 25 suitable vat colours, steamed for five minutes in air-free moist steam to effect reduction of the vat dyestuff, then developed by treatment with 1% solution bichromate of soda in 1% sulphuric acid at 60° C., followed by rinsing, 30 soaping at the boil and washing. In this case, the development of the vat colour on the warp threads is substantially inhibited, resulting in the production of shot effects.

Any other suitable thickening may be employed in place of the sizing mixture given 35 above.

**EXAMPLE 6**

Yarn in hank form may be treated as in 40 Example 5 on suitable machines as are commonly used for sizing hank yarn. Such yarn may then be woven or the like, as in Example 5 above.

**Case 4**

45 The fourth method of applying the invention consists in padding a cloth prepared from treated and untreated yarn, as in Case 3, instead of overprinting it. This is illustrated in the following example:—

**EXAMPLE 7**

Yarn prepared as in Example 5 or Example 50 6 is woven with untreated white yarn, and the resulting cloth padded by either of 55 the methods described herein in the examples illustrating Case 2.

**GENERAL**

Fabrics resisted as described above may be 60 used for any desired purpose, and materials resisted or sized may be woven in any suitable way, for example, according to British Letters Patent No. 292,415.

The examples are given by way of illustration only.

The preferred oxidizing agents are soluble alkaline salts of sulphonic acids of nitrated aromatic hydrocarbons, all of which are suitable for purposes of the present invention, particular attention being drawn to the nitrobenzene-sulphonic acid derivatives, especially the sodium salts of ortho- and meta-nitrobenzene sulphonic acids (resists salts L. or Ludigol). 70

Having now described our invention what 75 we claim as new and desire to secure by Letters Patent is:—

1. A process for securing the development of enolic ethereal salts of vat dyestuffs when these have had applied to them vat dyes and at the same time preventing the development of such vat dyes where they cover the enolic ethereal salt, which consists in the addition to the enolic ethereal salt of an oxidizing agent which is capable of serving as a resist towards vat dyes, and is substantially without effect on the enolic ethereal salt under the conditions used for applying the vat dye. 80

2. A colour resist process which consists in the application to textile fibres of mixtures containing enolic ethereal salts of vat dyestuffs, together with an oxidizing agent capable of serving as a resist towards vat dyestuffs, and being substantially without effect on the enolic ethereal salt under the conditions used for fixing vat dyestuffs, followed by application of ordinary vat dyestuffs, and then by subjection of the material to processes for the development of vat dyestuffs and enolic ethereal salts. 90

3. A process as claimed in claim 2, in which cloth is printed with a mixture containing the aforesaid oxidizing agent together with an ethereal salt of a vat dyestuff and a thickening agent, then steamed and overprinted with an ordinary vat dye and re-steamed to fix the vat dyestuff, the cloth being thereafter subjected to the usual process for fixation and development of the vat colour and the enolic ethereal salt. 105

In testimony whereof we have signed our names to this specification.

JAMES MORTON.

JAMES IVOR MORGAN JONES.

115

120

125

130